

Aug. 4, 1931.

I. R. VALENTINE

1,817,784

APPARATUS FOR PRODUCING LOW CARBON IRON

Filed Nov. 28, 1928

Fig. 1.



Fig. 2.



Inventor  
Irving R. Valentine  
by Charles E. Tullar  
His Attorney.

## UNITED STATES PATENT OFFICE

IRVING R. VALENTINE, OF ERIE, PENNSYLVANIA, ASSIGNOR TO GENERAL ELECTRIC COMPANY, A CORPORATION OF NEW YORK

## APPARATUS FOR PRODUCING LOW CARBON IRON

Application filed November 28, 1928. Serial No. 322,531.

The present invention relates to means for producing low carbon or perlitic cast iron in a cupola furnace. While perlitic iron has been produced heretofore, it has been customary in the production of such iron to regulate its carbon content by some means external to the cupola in which the iron was melted, such for example as a forehearth or externally heated furnace, or by preheat-  
10 ed molds into which the iron was cast.

It is one of the objects of the present invention to produce in a cupola melting furnace cast iron having a low carbon content and perlitic structure.

15 The novel features which I believe to be characteristic of my invention are set forth with particularity in the appended claims. The invention itself however will best be understood from reference to the following specification when considered in connection with the accompanying drawings in which Fig. 1 shows diagrammatically a cross section of a cupola melting furnace embodying the features of the present invention, while  
20 Fig. 2 is a cross section of the furnace taken on line 2—2 of Fig. 1.

Referring more particularly to the drawings, I have indicated at 1 a cupola melting furnace which comprises a metal casing  
30 2 lined with fire brick 3 and having a hinged metallic base plate 4 held in closed position by an iron post 5. The furnace 1 is of the ordinary cupola type and is provided with the usual wind boxes 6 and 7, tuyères 8 and  
35 9, slag hole 10 and tap hole 11. A brick wall 12 serves to support the cupola. The base plate 4 of the furnace is covered with a layer of sand 13 providing a hearth on which fire brick 14 or other suitable re-  
40 fractory material is laid so as to support a layer 15 of solid fuel such as coke or other carbonaceous material out of contact with the sand layer 13 and provide a space or reservoir 16 into which molten iron may  
45 settle and be held out of contact with the coke layer 15. It is desirable to extend the fire brick 14 about up to the slag hole 10.

In operation, the brickwork 3 and the lower coke bed 15 are heated by an oil burn-  
50 er or other suitable means until the brick-

work is red hot. The blast is then put on sufficiently to light the coke, and the cupola charged in the usual manner with alternate layers of coke and iron as indicated at 15 and 17 on the drawings. As the iron melts 55 it flows through the coke bed 15 and into the space or reservoir 16 in the base portion of the cupola and between the coke bed and the sand layer 13. In this manner the molten iron is in contact with the coke 15 60 for a very short period of time and the amount of carbon thus taken up by the molten iron is very small.

From a charge containing 30% scrap, 40% steel and 30% pig iron, castings have been 65 obtained which have a tensile strength of about 45,000 pounds per square inch and a Brinell hardness of 228, the content of the iron being substantially as follows:

|            | Per cent | 70        |
|------------|----------|-----------|
| Carbon     | 2.92     |           |
| Silicon    | 1.39     |           |
| Phosphorus | .40      |           |
| Manganese  | .40      |           |
| Sulphur    | .14      | 75        |
| Iron       | —        | Remainder |

In normal cupola operation the above charge would give iron having a tensile strength of approximately 32,000 pounds per square inch, a Brinell hardness of 180, a carbon content of 3.60% and a silicon content of 1.40%.  
80

Although I have employed fire brick, placed loosely in the base of the cupola to hold the coke bed out of contact with the sand layer and thereby provide a space in which the molten iron may be held out of contact with the coke bed, it will be clear that other constructions adapted to support or bridge the coke bed and permit the molten iron to flow therethrough may be employed if desired. Although it is possible with the arrangement shown to produce iron having a carbon content varying from 2 to 3%, 85 this content may be further reduced if desired by blowing air through the molten iron in the cupola.

What I claim as new and desire to secure by Letters Patent of the United States, is:  
100 1. A cupola melting furnace employing

solid carbonaceous fuel to melt the charge,  
said furnace comprising a hearth, refrac-  
tory means mounted on said hearth and  
adapted to support said carbonaceous fuel  
5 out of contact with the molten metal, and  
means for supplying a blast of air to said  
carbonaceous fuel.

2. A cupola melting furnace provided  
10 with a hearth portion and having a slag hole  
adjacent said hearth, and refractory means  
mounted in the furnace below said slag hole  
for supporting solid carbonaceous fuel and  
the metal to be melted, out of contact with  
the molten metal and means for supplying  
15 a blast of air to said carbonaceous fuel.

3. A cupola melting furnace having a  
hearth portion and a slag hole adjacent said  
hearth, refractory means mounted on said  
hearth and extending upwardly to a point  
20 adjacent said slag hole to support a charge  
of solid fuel and iron in the furnace and  
to provide a reservoir for the molten metal  
out of contact with said fuel.

In witness whereof, I have hereunto set  
25 my hand this 26th day of November, 1928.

IRVING R. VALENTINE.